

Sept. 14, 1937.

G. R. SHAW

2,092,815

CATHODE HEATER INSULATION

Filed Nov. 23, 1935

*Fig. 2*



*Fig. 1*



INVENTOR.

GEORGE R. SHAW

BY *Charles McClair*  
ATTORNEY.

## UNITED STATES PATENT OFFICE

2,092,815

## CATHODE HEATER INSULATION

George R. Shaw, Verona, N. J., assignor, by mesne assignments, to Radio Corporation of America, a corporation of Delaware

Application November 23, 1935, Serial No. 51,211

6 Claims. (Cl. 250—27.5)

My invention relates to indirectly heated thermionic cathodes and to heaters for such cathodes, and more particularly to refractory insulation for cathode heaters and to an improved method of insulating them.

In indirectly heated cathodes of a common type the heater wire of tungsten or similar metal has been insulated with a coating of substantially pure sintered alumina or of alumina mixed with a small percentage of silica or talc to act as a binder. The electrical leakage or conduction of current through the insulation has heretofore been tested by measuring the current which flows in response to a unidirectional potential between the cathode and the heater at operating temperature. By this test, heaters with the sintered alumina insulation have the least electrical leakage, usually less than 3 microamperes at 50 volts difference of potential. Such heaters are satisfactory for radio tubes in the conventional receiving circuits, but recently radio receiving circuits have come into use in which there may be alternating potentials as high as 100 volts or more and of high frequency, usually 1000 kilocycles or more, between the heater and the cathode. It has been found that the usual sintered alumina insulation, in spite of its very high resistance and very low leakage with unidirectional potential, has low impedance and permits appreciable leakage of current in response to alternating potential between the heater and the cathode. This leakage current is objectionable if excessive and may cause hum in the loud speaker of the receiving set.

One object of my invention is to provide an indirectly heated cathode in which the heater to cathode leakage is practically negligible at alternating potentials, even of high frequency, such as a kilocycle or more, between the heater and the cathode.

Another object of my invention is to provide a refractory composition with which a heater coil may conveniently be coated to provide an insulating layer having much higher impedance at all frequencies than the insulation heretofore available.

Still another object of my invention is to provide a method of insulating a cathode heater to make the impedance between the heater and the cathode very high and the leakage or electrical conductance negligible at alternating potentials such as are commonly used in radio receiving circuits and even at high frequencies.

Other objects and advantages of my invention

will appear from the more detailed description of my invention.

For a better understanding of my invention reference may be had to the accompanying drawing, in which Figure 1 is a longitudinal section of an indirectly heated cathode, and Figure 2 is a perspective view of the cathode heater.

The cathode assembly illustrated in the drawing is of a conventional type in general use, and comprises a tubular cathode 1 of nickel or similar metal coated on the exterior with oxides of high electron emissivity, such as the conventional coating of barium and strontium oxides. The cathode is heated by a heater comprising a wire 2 of tungsten or similar metal coiled into a reverse coil and mounted inside the tubular cathode. The heater wire is insulated from the cathode by a layer or coating of refractory insulation interposed between the wire and the cathode, preferably an insulating layer or coating 3 on the coiled tungsten wire 2. In use the heater is connected to a source of heating current, usually 60 cycle alternating current, which maintains the heater at a normal operating temperature considerably higher than the operating temperature of about 850° C. of the cathode 1.

For practical purposes an indication of the value of the heater to cathode leakage on alternating potential, and hence of the impedance of the insulation may be obtained by bringing the heater to normal operating temperature with 60 cycle alternating current, connecting the cathode to either end of the heater wire through a resistor of about 250,000 ohms, and measuring the voltage drop across the resistor in millivolts with a root mean square vacuum voltmeter having a grid resistor of about 1 megohm and connected to the resistor through a condenser. With the conventional heater designed to operate at 6 volts there is during this test an average difference of potential of about 3 volts at 60 cycles between the heater and the cathode, causing an impedance leakage current to flow through the insulation and through the resistor and produce the voltage drop which is measured and which is dependent on the value of the leakage current. The voltage thus measured I shall, in accordance with the custom in the art, refer to as the heater-cathode hum voltage. The absolute value of the heater-cathode hum voltage depends on the value of the resistor as well as on the value of the leakage current, but a resistor of 250,000 ohms gives values of heater-cathode hum voltage which are convenient and are in general use.

The impedance at high frequencies, such 1000

kilocycles, may also be measured with reasonable accuracy by a substitution method. One way of making this measurement is to use a radio frequency oscillator which oscillates at about 1000 kilocycles, and is very loosely coupled to a tuned circuit in which a voltage of about 0.4 or 0.5 volts is developed. To calibrate the testing set a resistor of known value, such as 1 megohm, and preferably of the metallized type, is connected across the tuned circuit, the circuit tuned to resonance, and the voltage across the resistor read by means of the vacuum tube volt meter above mentioned. This procedure is repeated with other resistors of different values to obtain 10 readings which correspond to resistors of different impedances. The heater cathode assembly to be tested is connected across the tuned circuit in place of the calibrating resistor, the circuit tuned to resonance while the heater is 15 kept at normal operating temperature, and the voltage of the tuned circuit across the cathode assembly is read. This reading, when compared with the readings obtained from the various resistors used in calibrating the test set, will show 20 with reasonable accuracy the impedance in megohms of the cathode assembly under test.

With the same test set a measurement of the current which flows between the heater and the cathode at high frequency may be obtained by 25 impressing between the heater and the cathode a constant bias or voltage of about 45 volts, either positive or negative, and then also impressing between the heater and the cathode the high frequency voltage obtained from the tuned 30 circuit of the test set. The bias of the heater to the cathode is varied to obtain minimum current, which is taken as the heater-cathode hum current at 1000 kilocycles.

Indirectly heated cathodes having heaters insulated with sintered alumina insulation may 40 show on the average on these tests heater-cathode hum voltages of seven or eight hundred millivolts or more, impedances of about 0.1 megohms, and heater-cathode hum currents of above 500 milliamperes. If the heater insulation is alumina 45 containing refractory binder such as silica or its compounds, the heater-cathode hum voltages and hum currents may be considerably greater and the impedance much less; but if the heaters are insulated in accordance with my invention, the heater-cathode hum voltages will on the average be only 10 to 50 millivolts, the impedances 50 from 1 to 3 megohms, or higher, and the heater-cathode hum currents from 20 to 100 milliamperes.

55 In accordance with my invention an insulating composition consisting of chemically pure alumina mixed with a small amount, such as  $\frac{1}{4}\%$  to 3%, of an additive material, preferably calcined barium carbonate, is applied to the heater wire and converted into the coherent layer or coating 60 by sintering the composition on the wire at high temperature. I have secured the best results in practice by adding to the alumina a compound of barium, particularly calcined barium 65 carbonate which has been fired in air. A convenient method is to powder both the alumina and the additive material and mix the powders thoroughly. This mixture may be further ground into a very fine powder, mixed with an 70 organic binder, the heater wire coated with it by well-known methods, such as spraying, and the coated heater wire fired, preferably in wet hydrogen, at about 1700° C. to 1800° C., which sinters the coating. The extent to which the mate-

rials are ground in preparing the insulation is not particularly critical, but the grinding is preferably continued until the average particle size, particularly in the final powder which is to be mixed with the binder, is about 1 to 5 microns. 5

In preparing the insulating material in accordance with my invention, I prefer to mix calcined and powdered barium carbonate, preferably chemically pure, with powdered aluminum oxide, as free as reasonably possible from impurities, especially alkalis, and usually referred to as chemically pure, fire the mixture in hydrogen at 10 1600° C. to 1700° C., and grind the fired mixture to a very fine powder.

One way of obtaining sufficiently pure alumina 15 from bauxite or similar ores is by the well-known Bayer process, in which in general the bauxite is treated in concentrated sodium hydroxide solution in water at 170° C. under pressure. The alumina goes into solution, the iron and other 20 impurities remaining as insoluble compounds. The solution is filtered off, and from it is obtained a precipitate consisting principally of aluminum trihydrate which, when heated in air at about 1200° C., is converted into alumina. 25 Alumina of substantially this degree of purity may also be purchased on the market as bauxite aluminum ore, concentrated, special purity, and said to contain not more than 0.2% of alkali. The alumina is fired at about 1600° C. in hydrogen, thereby shrinking it to maximum density 30 without sintering, and probably insuring that all of it is alpha-alumina.

The barium carbonate is preferably calcined 35 by firing it in air in a fire clay crucible at about 1100° C. for one hour. The calcined mass is ground into a fine powder by ball milling, and only that part of the powder which can be worked through a 150 mesh sieve with a paint brush is used. The calcined barium carbonate is of about 40 the same density as aluminum oxide, and will mix satisfactorily with it. It would seem that the barium compound could be added in the form of barium carbonate, but I have found that the results are so much better when the barium carbonate is first calcined and the barium is added to the alumina as calcined barium carbonate that 45 for commercial use the calcining of the barium carbonate may be essential.

The aluminum oxide powder is thoroughly 50 mixed with the calcined and powdered barium carbonate to form a mixture of which the powder obtained from the calcined barium carbonate constitutes from  $\frac{1}{2}\%$  to 5%, and preferably about 55 1% by weight. A ball mill is a convenient device for mixing powders. For example, about 800 grams of the powdered aluminum oxide and 8 grams of the calcined and powdered barium carbonate may be ball milled for about 2 hours with about 2500 grams of flint pebbles, to mix the 60 powders, and the mixture then fired at about 1600° C. in hydrogen for about one hour, preferably in molybdenum boats. The fired mixture is sieved through a 30 mesh sieve, and only the material which passes through the sieve rapidly is used. The fired and sieved mixture is then 65 ground into very fine powder in a ball mill with about three times its weight of mullite balls for about 18 hours and the powdered insulation is 70 ready for use.

The finely powdered insulation may be applied to the heater wire in practically the same way as the alumina insulation heretofore used. A convenient way is to mix the powdered insulation with a viscous organic binder, such as is com- 75

monly used in this art. I prefer to make a suspension of the powdered insulation by mixing it with about twice its weight of a binder such as nitro-cellulose dissolved in a solvent like amyrlac-  
5 etate. The insulation in suspension may be applied to the heater wire either by dipping or preferably by spraying to form a coating which should be uniform. The spray process for coating heater coils may be used on coils without a rigid core rod, if the coils are flexible enough so that the pressure from the spray gun moves them during the spraying to such an extent that the coating gets in between the turns. During the spraying all of the solid material in the coating  
10 preparation should be in suspension, the spray gun held close to the coils, and the spray adjusted to be sufficiently wet to obtain a smooth coating which adheres well to the wire and still be dry enough so that when adjacent turns stuck  
15 together by the coating are separated the coating does not break loose at the surface of either turn, but at the outer surface of the layers of coating. A wet spray is indicated by a glossy surface, while a dry spray is indicated by a dull or matte sur-  
20 face. The spray coated coil is dried in air, or preferably in an oven for three minutes at about 100° C., after which it is fired in a hydrogen or vacuum furnace, preferably in a molybdenum boat. The coated coils are fired for from four to  
25 eight minutes in the heating zone of the furnace maintained at a temperature of about 1700° C.

For a cathode heater of tungsten wire of a length and size suitable for operating at 6.3 volts and 0.3 amperes wound into a reverse coil about 25 mm. long and about 2 mm. in diameter, I prefer to use about 8 to 9 megohms of the coating preparation made and applied as above described.

Insulation consisting of alumina and about 1% of calcined barium carbonate forms on the tungsten wire of the finished heater a hard adherent coating, in which I find about 0.3% to 0.4% of barium by chemical analysis, indicating that roughly about 60% of the metal in the added material is lost during the manufacture of the insulation as above described. Somewhat the same percentage of loss occurs with other amounts of calcined barium carbonate so that the percentage of barium found by analysis may range from  $\frac{1}{8}\%$  to slightly over 1%. If the manufacture of the insulation is carried on under conditions such that there is less loss of the added metal, the percentage of added metal compound may be correspondingly reduced, and if none were lost, the addition of about 0.4% of calcined barium carbonate would mean the presence of the desired 0.3% barium in the sintered insulation of the finished heater. I have not determined in what form the barium found by chemical analysis is present in the insulation, but it is not present as metal, but as some refractory barium compound stable at the firing temperature, and is probably combined in some way with alumina, perhaps as a barium aluminate.

I have found that in practice the best and most consistent results are obtained with calcined barium carbonate added to the alumina. An addition of about 1% of calcined barium carbonate produces insulation with which a heater can be made having a heater-cathode hum voltage of from 10 to 50 millivolts when measured as above described, and the results are sufficiently consistent and controllable to permit use of the in-

sulation in commercial production. For practical purposes the lower and upper limits for the calcined barium carbonate in insulation prepared as above described appear to be about 0.1/2% and 3%. Insulation outside these limits has much higher heater-cathode hum voltages on the test above described than insulation within these limits. Calcined carbonates of calcium, strontium, or magnesium may be used instead of calcined barium carbonate with fairly good results if suitable amounts are used. Lithium carbonate acts much the same as barium carbonate and may be used in much the same way and in much the same proportions.

What I claim as new is:—

1. An indirectly heated cathode assembly comprising a tubular cathode sleeve coated on the outside with oxides of high electron sensitivity, a reversely coiled tungsten wire inside said cathode sleeve, and a coherent insulating coating on said wire consisting of chemically pure alumina and of a refractory oxygenic barium compound from  $\frac{1}{4}\%$  to 1% of the coating by weight of barium and having at normal heater operating temperature a heater-cathode hum voltage of less than 100 millivolts.

2. An indirectly heated cathode assembly comprising a cathode having a coating of electron emissive oxides, and a heater for said cathode comprising a wire of high melting point metal insulated from said cathode by coherent insulation containing an oxygenic barium compound and of which  $\frac{1}{4}\%$  to 1% of the coating by weight is barium and the remainder chemically pure alumina, and having at normal heater operating temperature sufficiently high impedance between said heater and said cathode to produce a heater-cathode voltage ranging between 10 and 50 millivolts.

3. A heater for indirectly heated cathodes comprising a heater wire of high melting metal, and a coherent sintered insulation coating on said wire of which substantially 99% is chemically pure alumina and the remainder an oxygenic barium compound stable at 1700° C. and containing from  $\frac{1}{4}\%$  to 1% of the coating by weight of barium by chemical analysis.

4. An indirectly heated cathode heater comprising a tungsten wire, and a sintered coherent insulating coating on said wire consisting of chemically pure alumina and an oxygenic barium compound stable at 1700° C. and of which 0.3% to 0.4% by weight of the coating is barium.

5. An indirectly heated cathode heater comprising a tungsten wire, and a sintered coherent insulating coating on said wire consisting predominantly of chemically pure alumina and the remainder of an oxygenic compound of a metal selected from the group of alkaline earth metals and lithium, said metal being  $\frac{1}{4}\%$  to 1% of the coating by weight and said compound being stable at 1700° C.

6. An indirectly heated cathode assembly comprising a cathode coated with electron emissive oxides, and a heater for said cathode comprising tungsten wire and a coherent insulating layer interposed between said cathode and said wire consisting predominantly of chemically pure alumina and the remainder a stable and refractory oxygenic compound of barium containing from  $\frac{1}{4}\%$  to 1% of the coating by weight of barium.

GEORGE R. SHAW.